

May 15, 1928.

1,669,506

H. C. J. DEEKS

PHOTOGRAPHY

Filed Oct. 1, 1924

*Fig. 1*



*Fig. 2*



*Fig. 3*



*Fig. 4*



Inventor  
Hiram C.J. Deeks.

By his Attorneys  
Emory Booth Murray & Palmer

Patented May 15, 1928.

1,669,506

# UNITED STATES PATENT OFFICE.

HIRAM C. J. DEEKS, OF SEA CLIFF, NEW YORK.

## PHOTOGRAPHY.

Application filed October 1, 1924. Serial No. 741,060.

Prior to making the present invention, I had employed the color pigments described and patented in my Letters Patent No. 1,430,061 dated, September 26, 1922 to produce colored gelatin reliefs from color-separation negatives, the gelatin reliefs then being combined, i. e., superposed in register, to produce a photograph in natural colors.

The present invention is the outgrowth of 10 my efforts to simplify the process by which that result was reached.

The combining and sticking together of three monochromes to produce a photograph in natural colors has never been a simple 15 operation. In my former process, to which I have just referred, the gelatin reliefs (produced with a bichromate sensitizer) were very delicate while wet and for that reason had to be thoroughly dry before any attempt 20 could be made to combine them. That meant considerable delay before any final result could be reached; and moreover, since the registration of the gelatin reliefs could only be effected after they were dry, special 25 apparatus had to be provided to permit the gelatin reliefs to be separated after registration for the application of moisture for sticking, and then be brought together again and sealed in exact registration. In addition to 30 these requirements, a long exposure with a high-powered arc lamp was required to print upon the bichromated gelatin which substantially added to the cost. And finally, the bichromated gelatin tissue itself would 35 not keep for any length of time but required almost immediate use. All of these things taken together multiplied the cost and difficulties of the process, necessitated a long and careful combining operation before any picture 40 could be seen, and thus greatly limited the availability of the process for both amateur and commercial use.

In my efforts to simplify that process, I have discovered that by embodying my pigments in a silver-gelatin emulsion and exposing and treating the same in the manner hereinafter described, I can produce colored gelatin reliefs so tough as to be easily registerable, one upon another, while still wet; 45 and this enables me to do away entirely with any apparatus for registration and combining the three monochromes and also reduces

very substantially the time required to produce and finish a photograph in natural colors since it is no longer necessary to wait for 55 each of the monochromes to dry before combining them together.

I have also discovered that any wet gelatin relief prepared, as hereinafter described, from my colored silver-gelatin film mounted 60 on a very thin celluloid backing, appears to thoroughly dry out although held tightly compressed between two layers of celluloid, one layer being the original backing upon which said relief was made and the other the 65 backing of an adjacent relief with which the first is combined in register; and also that when so combined perfect optical contact may be obtained between the reliefs to produce true color blending. It results, therefore, that no 70 transfer of the color films from one backing to another is required, but the reliefs may retain their original backing throughout without producing any defects either in the optical properties of the finished picture or 75 in the drying of the reliefs which, when dry, remain thoroughly and permanently united together.

Instead of employing a yellow colored pigment made in accordance with my aforesaid invention, for the yellow relief, in my present improved process I found it desirable to use chrome-yellow inasmuch as this is faster to light than any known yellow dye capable of employment in manufacturing my 80 own color pigments; and I discovered that with this chrome-yellow the gradations of the yellow relief more accurately represented the gradations of the negative than in the case of the red and blue reliefs. That led to 85 the discovery that by incorporating chrome-yellow in both the red and blue reliefs, in addition to the normal amounts of my red and blue colored pigments respectively, I was able to produce much more accurately the 90 gradations of the red and blue printing negatives than had been possible without the admixture of the chrome-yellow; and, in addition, I discovered that the clearing bath employed for clearing the relief after developing and bleaching, as described hereinafter, would also, if the reliefs were allowed to remain therein long enough, dissolve out the chrome-yellow in the end. In 95 100

this way, I found that I was able to reproduce accurately in all three gelatin reliefs the gradations of the negative without adding any additional step to the process as a whole.

From the foregoing it will be understood that the simplifications of my former process have been brought about through the embodiment of my color pigments in a silver-gelatin film; and I will now describe how this film is produced and used. I may say here that my improved film may be developed in a manner similar to that of a bromide print and then treated to harden the gelatin where the silver has been blackened, with the result that the unhardened gelatin may be washed away and the blackened silver bleached out so as to leave a pigmented gelatin positive in relief.

In manufacturing the film a silver-bromide emulsion is prepared in the customary manner but having as large a proportion of silver-bromide therein as will not incur liability of precipitation and, preferably, the proportions are such that the emulsion will contain about 11 per centum of gelatin. This proportion of gelatin is somewhat higher than usually used in coating celluloid film; but the celluloid which I prefer to use is much thinner than that ordinarily used for similar products and I have found it advisable to have a more viscous emulsion so that the coating will lie more evenly and without streaks on a very thin backing of celluloid.

Ordinarily, a gelatin-silver emulsion is permitted to stand several hours while being maintained at a high temperature, this process or step in the making of the emulsion being termed, "digesting." The digesting process adds to the speed or sensitivity of the emulsion, but it also renders it somewhat unstable and lowers its keeping qualities, and this is especially so if my color pigments are incorporated therein. Moreover, a fast emulsion is less desirable for my purpose for many reasons, although of course it is possible to obtain fair results even with a fast emulsion. Preferably, therefore, I dispense with digesting the emulsion so that when it is mixed and ready I immediately add my colors.

For this purpose I take 130 c. c. of a twelve per cent gelatin solution and place the same in a two gallon ball-mill. I then turn the mill over a few times so that the balls are covered with the gelatin solution and then add 53 grams of my transparent blue pigment and 27 grams of chrome-yellow. For a more particular description of my transparent pigments I refer to my Letters Patent aforesaid where a complete description thereof is given, it being sufficient to note here that said color pigments are produced by spraying a dyed solution of a

resin, such as sandarac, in alcohol and collecting the fine impalpable powder which results. The mill is then closed and allowed to grind for twenty minutes, after which 4000 c. c. of the silver emulsion previously prepared and kept in liquid form by continuing the temperature at 94° F., is added and the mill again allowed to revolve for ten minutes more. The coloring matter has now become thoroughly mixed with the emulsion and the mixture is poured from the mill, filtered through cloth, and poured into the pan of the coating machine.

The red and yellow colors are ground and mixed with the same amount of emulsion as for the blue color but I take 47 grams of my transparent red and 33 grams of chrome-yellow for the red color and 50 grams of chrome-yellow for the yellow color, the chrome-yellow being the only pigment used for the yellow.

In the accompanying drawings I have illustrated by views of exaggerated dimensions, the structure of color sheets prepared in accordance with my invention and also a three color photograph produced from said sheets. In said drawings Figure 1 illustrates the several sections of my blue sheet; Figure 2 the several sections of my red sheet; Figure 3 the several sections of my yellow sheet; and Figure 4 the several sections of a complete photograph formed from the several sheets upon a paper back laid upon a glass plate.

Before applying the coatings of color the celluloid should preferably be coated with a substratum on both sides,—the usual practice adopted in similar coating operations in order to make the emulsion adhere sufficiently to the celluloid. Such a sub-stratum may be the usual mixture of gelatin dissolved in acetic acid and then mixed with alcohol. The blue coating is applied to the celluloid having only the sub-stratum as described above; but the celluloid which is to be coated with the red emulsion and the celluloid which is to be coated with the yellow emulsion I first back with what I call a "sticking coat" so that when the yellow and red films are laid the celluloid in each case is coated on one side with the pigmented emulsion and on the other side with this "sticking coat." The mixture for the latter is as follows:

|                         |           |
|-------------------------|-----------|
| Water                   | 7000 cc.  |
| Gelatin                 | 490 grams |
| Acetic acid             | 90 cc.    |
| 3% chrome-alum solution | 560 cc.   |

The object of the "sticking coat", as will be seen later, is to stick the three monochromes together to form the final picture. Hence it is obvious this coating must be insoluble in hot water after it is dry since, if it were not, it would not withstand the

hot water bath which is used as part of the treatment in making the positive reliefs or monochromes presently to be described. When the "sticking coat" is dry the red or 5 yellow emulsion is coated on the other side in the usual manner.

I have already said that I prefer to use the thinnest celluloid procurable; and at the time of the application for this patent I 10 find that celluloid of .003 inches thick to be satisfactory. One reason why the celluloid should be as thin as possible is to permit the wet reliefs to dry while they are held tightly compressed between two layers of 15 celluloid as is the case when the combining of the three monochromes has been completed. I have found that this drying appears to take place through the celluloid and that at the end of about twenty-four hours 20 after combining, the reliefs seem to be thoroughly dry and firmly adhered together. Another reason for employing very thin celluloid is to maintain the three gelatin reliefs as closely together as possible and thus 25 avoid any parallax effect; moreover, on account of the somewhat yellowish color of the celluloid, it is desirable that it be very thin in order to interfere as little as possible with the clear rendition of the whites of the 30 picture.

The incorporation of chrome-yellow, I have found, helps to produce the correct relief gradations in the gelatin, that is, to 35 make them correspond to the tone values of the negative and hence enables me to produce exact duplications of colored prints. Besides this, the incorporation of chrome-yellow enhances the keeping qualities and prevents fogging in that its opaque nature 40 interferes with the penetration into the film of any dangerous light during the operations of manufacture and use; for a sufficient duration of exposure of any light-sensitive silver-emulsion to any so-called "safe" 45 red or green light will cause it to become light struck and while such fogging is to be avoided in ordinary black and white photography, it is much more objectionable in 50 color work because all fogging is represented in the finished picture by an entirely 55 visible color pigment deposit.

Moreover, the use of chrome-yellow also 60 helps to control the sensitiveness of the emulsion. The addition of a larger amount 65 of chrome-yellow to the red emulsion than to the blue, physically decreases the effect of the extra sensitiveness chemically produced by the red pigment and further decreases it so as to compensate for the desensitizing effect chemically produced by the 70 blue pigment. The proportion of chrome-yellow in the red and blue mixtures together with the proportions of red and blue pigment used, may thus be so adjusted as to 75 render the two mixtures of somewhat near

equal sensitiveness to each other and to the yellow mixture wherein chrome-yellow is used as the sole color pigment and has no chemical effect either to increase or decrease the sensitiveness of the emulsion. It will 80 be understood, of course, and will be explained later on, that all of the chrome-yellow in the red and blue reliefs is dissolved out and, unlike the case of the yellow relief, 85 forms no part of the color pigment in those reliefs when they are ready to be combined. It may be possible, therefore, to use, in the case of the red and blue pigments, some other opaque dissolvable matter to keep under control the penetration of the light 90 action and so produce the relief gradations (and therefore the tone values) in accordance with those of the negative.

From a practical standpoint, it is quite important to have the blue, red and yellow 95 emulsions all of the same, or as nearly the same, sensitiveness as possible so that with a set of three-color separation negatives of equal density the same exposure may be given to each because, if the operator in 100 making the three exposures has to take into consideration three printing sheets having a different sensitiveness-ratio in addition to three negatives having another different ratio or density the difficulty of procuring 105 accurately exposed and balanced color prints becomes obvious.

For the same reason, it is important that the emulsion shall not be too fast as I have already stated; for the faster the emulsion, 110 the less dependable the results. It is far more important that my improved pigmented emulsion should have plenty of latitude in exposure, no tendency to fog if developed at higher than normal temperatures 115 and have good keeping qualities than that the emulsion be fast; and by manufacturing the film as described above, I have found that an absolutely dependable product may be obtained with a substantial latitude of 120 exposure, development and other required treatment.

I have found that the incorporation of chrome-yellow in a silver-gelatin emulsion gives the emulsion a wonderful latitude of 125 exposure. It seems almost impossible to overexpose such a film while no additional step is introduced to the process of making a negative since the chrome-yellow is dissolved out at the same time as the unblackened silver in the ordinary hypo fixing bath.

With respect to the "sticking coat" described above, I have found that without this insoluble gelatin coat there appeared to be, in the lighter portions of the combined and finished print where very little pigmented gelatin remained, an interfering reflection of light which prevented the proper viewing of the combined colors in those portions. This did not seem to be caused by a layer of 130

air as no air space was ever found on analysis; and hence I have concluded it was probably caused by the contact of celluloid upon celluloid, producing a light reflecting surface which is not present when a "sticking coat" of gelatin is employed as described. I refer, therefore, to this improvement as not only enabling the reliefs to be stuck together conveniently, but as producing perfect optical contact when so united. Moreover, I point out that this result would not be practicable if soluble colors were used, that is to say, if the reliefs were dyed and then placed in contact with the wet "sticking coat"; for the dyes would immediately run out of the gelatin into the "sticking coat" the moment registration was attempted, and the entire "sticking coat" would become permeated with dye and the dye would be withdrawn from the parts of the picture where required to produce the proper effect. But with my special transparent though insoluble pigments, to which I have referred and in which the dye is retained by the resin and hence cannot be absorbed or drawn out of the reliefs by water or moist gelatin, the "sticking coat" has no effect whatever upon the color and the result sought is perfectly practicable.

Now, a brief explanation of the use of my improved color films will be given. It will be understood, of course, that in printing upon these films from three-color separation negatives, the negative taken through the green filter is printed onto the red film, the negative through the red filter onto the blue film and the negative through the violet filter onto the yellow film. For contact printing, the negative is first put into the printing frame with the emulsion side inwards as in ordinary printing. The film containing my improved emulsion is then inserted with the shiny or celluloid surface next to the negative because the exposure is made through the celluloid and not on the surface of the emulsion. For projection printing, a printing frame is still used but plain glass is put in place of the negative. The three negatives are successively exposed on their corresponding films and then developed, the exact exposure times being determined according to the density of the negatives but easily determined after a little practice.

The three prints are then preferably developed together for the same length of time, care being taken that they are not exposed any longer to dark room light than is absolutely necessary. After development they are rinsed and then immersed for ten minutes in a fixing solution. The three prints are now washed in running water for at least fifteen minutes; and it is very important that this washing be thorough and that the emulsion side be no touched during

that time. After washing, the prints are transferred to a bleach-hardening bath which causes the black image to disappear in about three minutes. The action of this bath is to harden and render insoluble the gelatin of the film in exact proportion to the amount of blackened silver of the image and, at the same time, the blackened silver is bleached or changed into whitish silver salt.

Next, the three prints are transferred directly to a warm water bath of about 100° F., until the soluble gelatin dissolves away, during which time the film surface should not be touched. This treatment requires from fifteen to twenty minutes and when complete the positive image will appear in color clearly visible. After the warm water washing the red and blue reliefs are immersed in a clearing solution for fifteen minutes or until the yellowish and greenish tint has disappeared from the shadows. This clearing solution removes the remaining silver and also the chrome-yellow. The yellow relief must not be put in the clearing solution but instead should be immersed for two minutes only in a fixing solution the same as was used directly after the developing operation.

The three reliefs are now immersed in cold, running water for about five minutes and then are ready to be combined in register while still wet upon white paper in the following manner: Take a sheet of glass about one inch longer and wider than the size of the film and a piece of white paper cut the same size as the color-sheet. The paper should be thin and have a smooth surface. The paper is placed next to the glass plate and both are held together under water for about five seconds to allow the paper to become thoroughly soaked. They are then taken together from the water and allowed to drain for a few seconds keeping the paper in the center of the plate. The plate with the paper upon it is now placed again under water and at the same time the yellow positive relief is brought into position under water on the paper, the color side being next to the paper. The plate with the paper and yellow positive together are now slowly withdrawn from the water in such manner that no air bubbles are retained between, and the surplus water is squeegeed out. The glass plate with the yellow relief thereon is again placed in the water and the red relief is brought into contact with the color side next to the yellow one and the plate is then withdrawn from the water as before. The red relief can now be slid into perfect register with the yellow relief by holding the glass plate with the fingers and using the thumbs at opposite edges of the red relief. All of the reliefs are quite tough and hence, though wet, they are not affected in the least by this treatment. When regis-

tration has been effected the surplus water is squeegeed out as before, care being taken not to disturb the register by squeegeeing; but, if the register has been disarranged it can be corrected by further sliding of the red relief. The same procedure is repeated for the blue relief.

The complete image is visible at once in natural colors at this point; but before the complete print is finished it must be allowed to dry, drying causing the three elements of the picture to thoroughly and permanently adhere together. For this it is preferable to seal the edges of the print upon the glass with gummed paper tape. This prevents curling up and separating during drying. Drying requires about twenty-four hours without any change taking place in the picture, after which the print is removed from the glass by cutting through the tape along the edges of the print with a sharp penknife.

I have found it particularly desirable to use the following solutions to obtain the best results and hence I append them hereto.

25

*For the developer.*

|                                          | Tray                       | Tank   |
|------------------------------------------|----------------------------|--------|
| Mono-methyl-p-aminometa-cresol-sulphate. | 92 grains or 6 g.          | 1½ oz. |
| A                                        |                            |        |
| Sodium sulphite (dry).                   | 1 oz. 34 grains or 30.5 g. | 8½ oz. |
| Potassium bromide.                       | 14 grains or 1 g.          | ¼ oz.  |
| Water.                                   | 16 oz. or 450 c. c.        | 1 gal. |
| B                                        |                            |        |
| Sodium carbonate (dry).                  | 400 grains or 26 g.        | 7½ oz. |
| Water.                                   | 16 oz. or 450 c. c.        | 1 gal. |

35 The above solutions will keep well in stoppered bottles. For use mix together equal quantities of A and B.

*For the fixing solution.*

|        | Tray                | Tank    |
|--------|---------------------|---------|
| Hypo.  | 3 oz. or 85 g.      | 1½ lbs. |
| Water. | 16 oz. or 450 c. c. | 1 gal.  |

45 A hypo bath containing acid, alum, or other ingredients should not be used.

*For the bleach-hardening bath.*

|                         | Tray                      | Tank    |
|-------------------------|---------------------------|---------|
| Copper sulphate (C. P.) | 1½ oz. or 37 g.           | 10½ oz. |
| Potassium bromide.      | 1½ oz. or 37 g.           | 10½ oz. |
| Ammonium bichromate.    | 143 grains or 9.25 g.     | 2½ oz.  |
| Acetic acid (glacial).  | 210 minimis or 12.5 c. c. | 3½ oz.  |
| Water.                  | 16 oz. or 450 c. c.       | 1 gal.  |

Dissolve each chemical completely before adding the next one in the order given. The dissolving of the copper sulphate (which takes several minutes) may be hastened if the crystals are powdered and if the water is hot.

*For the clearing solution.*

|        | Tray                | Tank    |
|--------|---------------------|---------|
| Hypo.  | 4 oz. or 113.5 g.   | 1½ lbs. |
| Water. | 16 oz. or 450 c. c. | 3 qts.  |

When dissolved add the following (first thoroughly dissolving it).

|                           | Tray               | Tank   |
|---------------------------|--------------------|--------|
| Potassium meta-bisulphite | ½ oz. or 10.5 g.   | 2½ oz. |
| Powdered chrome-alum      | ½ oz. or 7 g.      | 1½ oz. |
| Water.                    | 4 oz. or 115 c. c. | 24 oz. |

I claim as my invention:

1. A silver-halide-sensitive emulsion containing transparent color pigments and chrome - yellow distributed uniformly throughout the emulsion.

2. A silver-halide-gelatin emulsion containing chrome-yellow distributed uniformly throughout the emulsion.

3. A photographic film comprising a transparent backing, a sensitive coating on one side containing fine transparent color pigments insoluble in water and a sticking coat on the other.

In testimony whereof, I have signed my name to this specification this 30th day of September, 1924.

HIRAM C. J. DEEKS.